

# UNITED STATES PATENT OFFICE.

JEAN FRANCOIS PUTTAERT AND HENRY F. J. PUTTAERT, OF SAN FRANCISCO,  
CALIFORNIA.

## MANUFACTURE OF PULP AND PAPER FROM GARBAGE.

1,294,163.

Specification of Letters Patent.

Patented Feb. 11, 1919.

No Drawing.

Application filed December 12, 1916. Serial No. 136,446.

*To all whom it may concern:*

Be it known that we, JEAN FRANCOIS PUTTAERT and HENRY FRANCIS JOSEPH PUTTAERT, subjects of the King of Belgium, residing at the city and county of San Francisco and State of California, have invented new and useful Improvements in Manufacture of Pulp and Paper from Garbage, of which the following is a specification.

10 Our invention relates to the manipulation of garbage in such a manner as to separate it into various useful compounds after deodorizing it.

It consists particularly in the preparation of a pulp which may afterward be converted into cardboard, binder board roofing papers, felt papers, and generally into kindred useful forms.

20 The garbage being first collected, all hard substances, such as stones, glass, iron, tin cans, bones, and the like, are separated and removed. The remaining material is then passed through suitable crushing machinery and reduced to a coarse pulp which may contain as much as fifty per cent., more or less, of moisture. The stock thus produced is passed through a press and a considerable proportion of the moisture is extracted. From this extract by suitable processes, useful oils or greases can be extracted. The solid residue may retain from ten to twenty per cent. of moisture, or sufficient to enable it to be further worked.

35 This pulp is then placed in suitable boilers with any desired alkaline or other reagents, and is then boiled until thoroughly deodorized and deprived of remaining

grease and undesirable substances. It is then thoroughly washed and bleached and is transferred to a beating or like engine, in 40 which it is reduced to a clean fibrous pulp, which by subsequent proper manipulation may be transformed into card, binder, or roofing boards, or like structures for kindred uses.

45 This is all effected without smoke, smell or gases of any kind.

Having thus described our invention, what we claim and desire to secure by Letters Patent is—

50 1. The process of reduction and preparation of garbage, consisting in first removing all deleterious hard substances, then crushing the resulting mass, expressing a proportion of moisture, boiling the residue 55 with suitable alkaline reagents, and forming a fibrous pulp.

2. The process of manufacturing cardboard and the like from garbage, consisting in first removing deleterious hard substances, crushing and removing a percentage of moisture from the remainder, boiling the resultant mass with an alkaline reagent, washing and bleaching and reducing to a fibrous pulp, and finally converting said pulp into 60 65 dry sheets.

In testimony whereof we have hereunto set our hands in the presence of two subscribing witnesses.

JEAN FRANCOIS PUTTAERT.

HENRY F. J. PUTTAERT.

Witnesses:

JOHN H. HERRING,  
W. W. HEALEY.